

Nov. 10, 1925.

1,561,067

M. FERREE ET AL

PHOTOTELEGRAPHIC TRANSMITTING PLATE

Filed Jan. 31, 1925



INVENTORS  
Marion Ferree  
& Joseph Wissner  
BY  
Moe & Blum  
ATTORNEYS

## UNITED STATES PATENT OFFICE.

MARVIN FERREE, OF NEW YORK, N. Y., AND JOSEPH WISSMAR, OF CLEVELAND, OHIO, ASSIGNEES TO PACIFIC AND ATLANTIC PHOTOS, INC., OF NEW YORK, N. Y., A CORPORATION OF NEW YORK.

## PHOTOTELEGRAPHIC TRANSMITTING PLATE.

Application filed January 31, 1925. Serial No. 5,954.

*To all whom it may concern:*

Be it known that we, MARVIN FERREE and JOSEPH WISSMAR, citizens of the United States, residing in the city, county, and State of New York, and in the city of Cleveland, county of Cuyahoga, and State of Ohio, respectively, have invented certain new and useful Improvements in Phototelegraphic Transmitting Plates, of which the following is a specification.

This invention relates to a new and useful improvement in making broken tone plates for use in transmitting pictures by a series of electrical pulses.

It has been known to make a broken tone duplicate of a picture by means of a series of spaced dots, these dots being composed of insulating material, and being arranged upon a conductive plate. By connecting the conductive plate to one terminal of a source of electricity, and by connecting the other terminal of said source of electricity to a needle having a fine point, the circuit was made and broken as the needle and plate were moved relatively to each other.

Pictures transmitted by the use of a broken tone plate made as before described, were often coarse because of the grained effect so that the reproduction was inferior.

According to this invention the broken tone picture consists of a series of lines which are preferably parallel and which are of varying width. These lines are composed of insulating material located upon a plate made of copper or other material which will conduct electricity.

The drawing shows a preferred embodiment of this invention.

The picture to be reproduced is first placed in front of an ordinary camera so that a negative can be made thereof. This negative is made upon an ordinary transparent glass plate either wet or dry. Before the negative impression is made, a transparent grating having a series of parallel opaque lines thereon is placed in the camera before the negative so that the negative image consists of a series of parallel opaque lines of varying thickness and the continuous tone of the picture to be reproduced is thus duplicated in what may be called broken tone.

The spacing of the opaque lines may vary

and we do not wish to limit ourselves to any particular spacing but we have found that a grating having sixty-five lines to the inch is satisfactory for reproducing ordinary photographs. The thickness of the said opaque lines may be equal to the distances between them but we do not wish to limit ourselves to any particular type of grating. We have found the use of gratings having parallel lines to be far superior to gratings having lines crossing each other for this particular purpose because the points of light in the picture to be reproduced are, according to our invention, spread out only in the vertical direction instead of being spread out both in the vertical and in the horizontal direction. Hence, the transmitting plate which will be later described does not consist of a series of separated dots of insulating material. Experiments have shown that the improved transmitting plate made according to our process avoids the coarse pattern effect produced when the negative is taken through a grating having cross lines. We prefer to have the opaque lines of the grating held horizontally when the negative is taken. The negative thus produced is now used for making an enlarged positive by means of an ordinary camera. We prefer to make this positive twice as large as the negative of the original picture. This enlargement enables a superior transmitting plate to be reproduced. The enlarged positive thus produced is now printed upon a thin plate made of copper or other suitable bendable metal by means of an ordinary printing frame. This metal plate which may be called the transmitting plate is coated with a sensitive film comprising fish glue, ammonium bichromate and white of eggs. This coating is made of sixteen ounces of fish glue, one ounce of ammonium bichromate, six egg whites and either seventeen or thirty-four ounces of water. These ingredients are thoroughly mixed and they are spread upon the highly polished surface of the copper plate. This coating is then dried, in which condition it is not very sensitive to daylight but is sufficiently sensitive to a powerful arc light used for printing thereon from the enlarged positive. After the copper plate has been exposed, it is washed in cold water until the

portions of the coating which have not been acted upon by the light are washed away and the plate is then dipped in aniline dye which is absorbed by the remaining gelatine so as to furnish a reproduction of the image to see if the photographic work has been properly done. The plate is then washed to remove any surplus dye and it is then baked over a suitable flame or the like 10 until the adhering coating has been transformed into a hard enamel-like material. After the enamel has been formed, the plate is cleaned by rubbing it with a mixture of acetic acid and salt as this eats away any 15 of the coating which does not correspond to the image so as to produce clean bright copper lines between parallel lines of enamel of varying width.

The plate thus formed can now be bent 20 if desired so that it now has a cylindrical shape and the bent plate can now be placed upon the drum of a transmitting machine of any ordinary and well-known type.

A device of the type in which this plate 25 is adapted to be used is shown in U. S. Patent No. 1,529,473.

A preferred embodiment of this invention has been described but it is clear that numerous changes and omissions could be 30 made without departing from its spirit.

Experience has shown that if the metal plate is developed in the ordinary manner, then the portions or strips of the copper plate intermediate the lines of insulating 35 material are not clean and bright, because some of the insulating material remains on said strips. By treating the developed and baked plate with a weak acid, such as acetic acid, and with a mild abrasive, such as particles of salt, the undeveloped portion 40 of the coating is effectually removed. This results in the production of a clear picture, without any noticeable pattern or grain.

#### Claims:

1. A phototelegraphic transmission plate 45 made of metal, said metal plate having thereon a broken tone reproduction of the picture to be electrically transmitted, the said broken tone reproduction comprising a series of parallel lines of varying thickness, 50 the said lines being composed of hard insulating material, that portion of the copper plate intermediate the said lines of insulating material being free from the said insulating material. 55

2. A method of making a phototelegraphic plate for transmitting pictures by means of a series of electrical pulses which consists in making a negative of a picture to be reproduced through a transparent grating having a series of parallel opaque lines thereon so that the negative image thus formed has a series of parallel opaque lines of varying thickness, then making a positive from the said negative thus produced, 60 then printing with the said positive upon a coating of light sensitive glue located on a metal plate, then developing the said coating so as to wash away the portions which have not been acted upon by the light, then 65 baking the said coating so as to harden it and then removing any of the said coating which does not correspond to the image. 70

3. A method according to claim 2 in which the surplus coating is removed by rubbing 75 the coating with a mixture of acetic acid and salt. 75

4. A method according to claim 2 which consists in removing the surplus coating by washing it with a weak acid and a mild 80 abrasive. 80

In testimony whereof we hereunto affix our signatures.

MARVIN FERREE.  
JOSEPH WISSMAR.